

3,594,319

## ADDITIVES FOR FUEL ANTIOXIDANTS AND FOR LUBRICANTS

Heinrich Vollmann, Leverkusen, Heinrich Leister, Cologne-Stammheim, and Walther Lohmar, Bergisch-Gladbach, Germany, assignors to Farbenfabriken Bayer Aktiengesellschaft, Leverkusen, Germany

No Drawing. Filed Jan. 21, 1969, Ser. No. 792,788  
Claims priority, application Germany, Jan. 29, 1968,

P 16 44 897.8

Int. Cl. C10m 1/32; C10I 1/22

U.S. Cl. 252—51.5A

6 Claims

### ABSTRACT OF THE DISCLOSURE

Additives to lubricants and fuel antioxidants, consisting of or containing isoindoline compounds of the formula



in which R stands for an alkyl, isoalkyl or alkenyl radical with 7 to 20 carbon atoms.

The present invention relates to additives to lubricants and fuel antioxidants. More particularly it concerns additives to lubricants and fuel antioxidants consisting of or containing isoindoline compounds of the formula



(II)

in which R stands for an alkyl, isoalkyl or alkenyl group with 7 to 20 carbon atoms, preferably with 8 to 20 carbon atoms.

These isoindoline compounds have proved to be outstandingly effective as additives to lubricants and fuel antioxidants.

The preferred compounds of the Formula I are those in which R denotes an alkyl group with 12 to 20 carbon atoms. Compounds of the Formula I in which R is an alkenyl group with 18 carbon atoms have an especially high synergistic effect in fuel antioxidants.

As radicals should be mentioned for R for example: C<sub>10</sub>—C<sub>20</sub>-alkyl radicals such as the decyl-, dodecyl, tetradecyl-, hexadecyl- or octadecyl radical; C<sub>10</sub>—C<sub>20</sub>-isoalkyl radicals such as the 2,2-dimethyl-octyl-(1), 2,2-dimethyl-dodecyl-(3), 2,2-dimethyl-4-iso-butyl-heptyl-(4), 2,3-dimethyl-dodecyl-(3), 2,2-dibutyl-hexyl-(1), 3-methyl-heptadecyl-(17), or the 2,6,10,14-tetramethyl-hexadecyl-(16) radical; C<sub>10</sub>—C<sub>20</sub>-alkenyl radicals such as the decen-(1)-yl-(4), 2,6-dimethyl-decen-(1)-yl-(8), 2,6-dimethyl-dodecen-(2)-yl-(12), 4-methyl-pentadecen-(14)-yl-(1), octadecen-(9)-yl-(1) or the 2,6,10,14-tetramethyl-hexadecen-(14)-yl-(16) radical.

The isoindoline compounds to be used according to the invention are insoluble in water; some are crystalline compounds, some are viscous liquids. They can be obtained, for example, by condensing 1,3-diimino-isoindoline and suitable cyanoacetic esters in solvents as is described in Belgian Pat. 703,669. The compounds are ash-free and non-volatile and thus facilitate their incorporation with organic material. The compounds are readily

soluble in solvents, such as e.g. N-methyl-pyrrolidone and it is therefore possible to prepare also highly concentrated solutions with a view to better dosage.

The amounts in which the isoindoline compounds of the Formula I have to be used in any given case can easily be established by preliminary experiments; for use as additives to lubricants, amounts of 0.001—1.0 percent by weight, based on the weight of the lubricants, and for use as additives to fuel antioxidants, amounts of 3—10 percent by weight, based on the weight of the antioxidants, have usually proved sufficient.

With the aid of the isoindoline compounds of the Formula I it is possible substantially to improve lubricants of various types, particularly in respect of their resistance to oxidative attacks. This is mainly true of lubricants prepared from mineral oils and of lubricants of synthetic origin. For example, turbine, hydraulic, transformator and other highly refined industrial oils, soaps and fats, lubricating fats, but also synthetic polymers such as polybutenes and the like are, very effectively stabilised against attacks by air and oxygen. Compounds of the Formula I are also suitable for stabilising fats and oils of animal or vegetable origin.

The additives to lubricants to be used according to the invention are compatible with the majority of other additives to lubricants, for example, with detergents, agents for improving the stability of the lubricating film, and agents for improving the solidification point and the viscosity.

It is of special advantage to add the isoindoline compounds together with diphenylamines serving as antioxidants such as N-phenyl-N-isopropyl-p-phenylene-diamine or 4,4'-dimethylbenzyl-diphenylamine. A synergistic effect is thus achieved.

It is further possible with the aid of the isoindoline compounds of the Formula I substantially to improve the antioxidant effect of commercial antioxidants of various types, for example, of phenolic antioxidants, such as

2,6-di-tert.-butyl-4-methyl-phenol,  
2,4-dimethyl-6-tert.-butyl-phenol,  
2,6-di-tert.-butyl-phenol, and, in particular, of p-phenylene-diamine antioxidants, such as  
N,N'-diisopropyl-p-phenylene-diamine,  
N,N'-di-sec.-butyl-p-phenylene-diamine,  
N-phenyl-N'-isopropyl-p-phenylene-diamine,  
N-(1,3-dimethyl-butyl)-N'-phenyl-p-phenylene-diamine.

It is remarkable that the isoindoline compounds to be used according to the invention are compatible with most other additives to fuels, for example, with agents for increasing the resistance to compression and to anti-icing agents and agents against the formation of residues and vapour bubbles.

The surprisingly high effectiveness of the isoindoline compounds of the Formula I as additives to lubricants was established in the apparatus described by C. Kröger in the journal "Erdöl und Kohle," vol. 2 (1949), page 390. This apparatus consists of a reaction vessel with connected open-end mercury manometer.

The small flask of 12.5 ml. capacity is charged with 1 g. of mineral oil in which 0.001 g. of antioxidant have been dissolved, and with 0.1 g. of copper powder. The copper powder is added as oxidation activator. Before the manometer is connected, the air is driven out of the reaction vessel by means of oxygen and the flask is then placed on an oil bath at a constant temperature of 150° C. ± 0.5° C. A shaking device keeps the content of the flask in motion so that the copper powder is well dispersed in the oil sample mixed with the antioxidant, and the oil sample remains in good contact with the oxygen.

Due to the heating, the pressure in the apparatus rises very rapidly and reaches an excess pressure value of up to

190 mm. Hg after 3-4 minutes; it decreases again when the oxidation reaction starts. The maximum excess pressure value is set as zero. The decrease of pressure in the system caused by the consumption of oxygen by the system is measured at certain time intervals. The magnitude of the velocity of oxidation is characterised by the decrease of pressure in mm. Hg/min. The lower this quotient is, the more effective is the antioxidant.

As starting oil for the tests there was used a mineral oil with the following characteristics:

Density at 20° C: 0.897 g./ml.; neutralisation number: 0.06 mg. KOH/g. oil; aniline point: 89.5° C.; solidification point: -28° C.; viscosity at 20° C.: 205.0 cst.; ash after combustion: 0.005 percent by weight.

The following compounds were used as additives:

- 1,3-bis- $\alpha$ -pyridyl-imino-isoindoline (according to U.S. Patent specification No. 3,129,227) (A)  
 $C_{12}$ - $C_{14}$ -alkyl ester of 1-(cyanocarboxy-methylene)-3-imino-isoindoline (B)  
 1 - (cyano - carbocetylloxy - methylene) - 3 - imino - isoindoline (C)  
 $C_{12}$ - $C_{18}$ -alkyl ester of 1-(cyanocarboxy-methylene)-3-imino-isoindoline (D)  
 10% solution of (D) in N-methyl-pyrrolidone (E)  
 1 - (cyano - carbostearylloxy - methylene) - 3 - imino - isoindoline (F),  
 1 - (cyano - carbooctadecen - (9') - yl - (1') - oxy - methylene)-3-imino-isoindoline (G)  
 14% solution of (G) in N-methyl-pyrrolidone (H)  
 $C_{11}$ - $C_{19}$ -alkyl ester of 1-(cyanocarboxy-methylene)-3-imino-isoindoline (I)

Compounds B through I are isoindoline compounds of the present invention.

The test results obtained with various additives are assembled in Table I::

TABLE I

| Example                                                            | Velocity of oxidation, mm.<br>Hg/min. |
|--------------------------------------------------------------------|---------------------------------------|
| 1..... Base oil.....                                               | 0.813                                 |
| 2..... Base oil plus copper powder.....                            | 1.755                                 |
| 3..... Base oil plus copper powder plus 0.1 percent by weight (A)  | 1.150                                 |
| 4..... Base oil plus copper powder plus 0.1 percent by weight (B)  | 0.532                                 |
| 5..... Base oil plus copper powder plus 0.1 percent by weight (C)  | 0.561                                 |
| 6..... Base oil plus copper powder plus 0.1 percent by weight (D)  | 0.507                                 |
| 7..... Base oil plus copper powder plus 0.1 percent by weight (E)  | 0.556                                 |
| 8..... Base oil plus copper powder plus 0.1 percent by weight (F)  | 0.550                                 |
| 9..... Base oil plus copper powder plus 0.1 percent by weight (G)  | 0.400                                 |
| 10..... Base oil plus copper powder plus 0.1 percent by weight (H) | 0.384                                 |
| 11..... Base oil plus copper powder plus 0.1 percent by weight (I) | 0.500                                 |

The surprising synergistic effect of the isoindoline compounds of Formula I in fuel antioxidants was demonstrated in the bomb test for liquid fuels according to ASTM D 525-55 respectively DIN 51,780. According to this test, a test vessel of glass which has a capacity of 150 ml. and was previously cleaned and dried at 150° C., is placed in a carefully cleaned V2A-steel bomb. The steel vessel is charged with 50±1 ml. gasoline in which the desired amount of the antioxidant has been dissolved. The glass vessel is covered with a glass lid. The V2A-steel bomb is then sealed gas-tight with a lid. The lid of the steel bomb is fitted with a fine-control valve and a terminal which is connected via a capillary spiral to a recording manometer. The V2A-bomb is rinsed twice with oxygen at 7 atm. excess pressure in order to remove the air initially present. Oxygen is then again pressed in at 7.00 to 7.14 atm. excess pressure. The bomb thus charged is placed, without shaking it, in a water bath which has been heated to 100° C. and is kept briskly boiling. The

70  
75

content of the bomb is in communication with the recording manometer so that the course of the pressure as a function of time, i.e. the pressure-time curve, is graphically recorded.

The time in minutes which elapses from the start of the test to the detectable absorption of oxygen, i.e. the pressure drop, is stated as "induction period at 100° C.": the point of pressure drop in the pressure-time curve is the point which is preceded by a decrease of pressure of exactly 0.14 kg./sq. cm. within 15 minutes and followed by a decrease of pressure of at least 0.14 kg./sq. cm. within 15 minutes.

The test results obtained with the various additives are assembled in the following Tables II and III: in Table II the protection against oxidation achieved by various additives in thermally produced heavy cracked gasoline at 100° C.; in Table III, the protection against oxidation achieved by various additives in catalytically produced heavy cracked gasoline at 100° C.

The gasolines used for the tests had the following characteristics:

|                                          | Thermally produced heavy cracked gasoline | Catalytically produced heavy cracked gasoline |
|------------------------------------------|-------------------------------------------|-----------------------------------------------|
| Density at 20° C., g./ml.....            | 0.848                                     | 0.755                                         |
| Bromine number, g./100 g.....            | 52                                        | 83                                            |
| Diene content, percent by weight.....    | 8.1                                       | 3.3                                           |
| Carbon, percent by weight.....           | 90.6                                      | 86.8                                          |
| Hydrogen, percent by weight.....         | 9.4                                       | 13.4                                          |
| Non-aromatic, percent by weight.....     | 19.8                                      | 71.49                                         |
| Lower aromatics, percent by weight.....  | 74.8                                      | 21.86                                         |
| Higher aromatics, percent by weight..... | 5.4                                       | 6.65                                          |
| Gum before ageing, mg./100 ml.....       | 56                                        | 1                                             |
| Gum after ageing, mg./100 ml.....        | 10.400                                    | 2.104                                         |

The additives used were:

- 1 - (cyano - carbooctadecene - (9') - yl - (1') - oxy - methylene)-3-imino-isoindoline (A),  
 N-phenyl-N'-isopropyl-p-phenylene-diamine (B),  
 N - (1,3 - dimethylbutyl) - N' - phenyl - p - phenylene-diamine (C),  
 2,6-di-tert.butyl-4-methyl-phenol (D) and mixtures of A+B, A+C and A+D.

TABLE II

| Test                                           | Additive | Concen-<br>tration<br>(p.p.m.) | Induction<br>period<br>(min.) |
|------------------------------------------------|----------|--------------------------------|-------------------------------|
| 1..... A.....                                  |          | 10                             | 26                            |
|                                                |          | 50                             | 28                            |
| 2..... B.....                                  |          | 100                            | 48                            |
|                                                |          | 50                             | 115                           |
| 3..... Mixture of 1 part A plus 9 parts B..... |          | 100                            | 166                           |
|                                                |          | 50                             | 52                            |
|                                                |          | 100                            | 147                           |
|                                                |          | 100                            | 230                           |

TABLE III

| Test                                           | Additive | Concen-<br>tration<br>(p.p.m.) | Induction<br>period<br>(min.) |
|------------------------------------------------|----------|--------------------------------|-------------------------------|
| 4..... B.....                                  |          | 100                            | 811                           |
| 5..... Mixture of 1 part A plus 9 parts B..... |          | 100                            | 925                           |
| 6..... C.....                                  |          | 100                            | 772                           |
| 7..... Mixture of 1 part A plus 9 parts C..... |          | 100                            | 980                           |
| 8..... D.....                                  |          | 100                            | 469                           |
| 9..... Mixture of 1 part A plus 9 parts D..... |          | 100                            | 590                           |

What is claimed is:

1. Additives for fuels and lubricants consisting essentially of isoindoline compounds of the formula



in which R stands for an alkyl, isoalkyl or alkenyl radical with 7 to 20 carbon atoms.

2. Lubricant of improved oxidation stability comprising a natural or synthetic lubricant and an isoindoline compound of the formula



in which R stands for an alkyl, isoalkyl or alkenyl radical with 7 to 20 carbon atoms.

3. The lubricant of claim 2 comprising 0.001-1.0 percent by weight of the isoindoline compound based on the weight of the lubricant.

4. Antioxidant mixture of increased effectiveness for liquid fuels comprising a phenolic antioxidant or a p-phenylene-diamine antioxidant and an isoindoline compound of the formula



in which R stands for an alkyl, isoalkyl or alkenyl radical with 7 to 20 carbon atoms.

5. The antioxidant of claim 4 comprising 3-10 percent by weight of the isoindoline compound based on the weight of the phenolic or p-phenylene-diamine antioxidant.

6. The antioxidant of claim 4 wherein the p-phenylene-diamine antioxidant is a member selected from the group consisting of N,N'-diisopropyl-p-phenylene-diamine, N,N'-disec-butyl-p-phenylene-diamine, N-phenyl-N'-isopropyl-p-phenylene-diamine, N-(1,3-dimethylbutyl-N'-phenyl-p-phenylene-diamine.

#### References Cited

#### UNITED STATES PATENTS

- |    |           |        |                |         |
|----|-----------|--------|----------------|---------|
| 15 | 2,521,415 | 9/1950 | Schmerling     | 44-63   |
|    | 2,930,758 | 3/1960 | Tierney et al. | 252-50X |
|    | 3,129,227 | 4/1964 | VanVelzen      | 44-63   |
|    | 3,322,785 | 5/1967 | Fletcher       | 252-403 |

20 DANIEL E. WYMAN, Primary Examiner

W. J. SHINE, Assistant Examiner

#### U.S. CL. X.R.

25 44-63; 252-50, 403; 260-326.1